

# United States Patent

[11] 3,615,415

[72] Inventor **Eugene P. Gramza**  
Rochester, N.Y.  
[21] Appl. No. **821,513**  
[22] Filed **May 2, 1969**  
[45] Patented **Oct. 26, 1971**  
[73] Assignee **Eastman Kodak Company**  
Rochester, N.Y.  
Continuation-in-part of application Ser. No.  
586,648, Oct. 14, 1966, now abandoned,  
and a continuation-in-part of 674,006, Oct.  
9, 1967, now abandoned.

[56] **References Cited**  
UNITED STATES PATENTS  
3,052,540 9/1962 Greig..... 96/1.7  
3,110,591 11/1963 Stewart ..... 96/1.7  
3,141,770 7/1964 Davis et al. ..... 96/1.6 X  
3,250,615 5/1966 Van Allen et al. ..... 96/1.7  
3,251,687 5/1966 Fohl et al. ..... 96/1.7  
*Primary Examiner—George F. Lesmes*  
*Assistant Examiner—R. E. Martin*  
*Attorneys—W. H. J. Kline, J. R. Frederick and T. Hiatt*

[54] **METHOD FOR THE PREPARATION OF PHOTOCONDUCTIVE COMPOSITIONS**  
12 Claims, No Drawings  
[52] U.S. Cl. .... 96/1.6,  
96/1.7, 260/37, 260/34.2  
[51] Int. Cl. .... G03c 5/06  
[50] Field of Search. .... 96/1.6, 1.7;  
252/501

**ABSTRACT:** Multiphase heterogeneous compositions are formed from an organic dye and electrically insulating polymeric material. A solution of dye and polymer is prepared and subsequently subjected to high speed shearing. Electrophotographic layers can be prepared by coating the sheared solution to form the multiphase heterogeneous compositions. Such compositions which are useful as photoconductors or electrophotosensitizers are characterized by a radiation absorption maximum that is substantially shifted from the absorption maximum of a simple, untreated solution of dye dissolved in polymer.

**METHOD FOR THE PREPARATION OF  
PHOTOCONDUCTIVE COMPOSITIONS**

This application is a continuation-in-part based on application Ser. No. 586,648, filed Oct. 14, 1966 and Ser. No. 674,006, filed Oct. 9, 1967 now both abandoned.

This invention relates to electrography and to photoconductive compositions, elements and structures useful in electrophotography. In addition, this invention relates to providing novel electrophotographic compositions together with methods for their preparation and use.

Electrophotographic imaging processes and techniques have been extensively described in both the patent and other literature, for example, U.S. Pat. Nos. 2,221,776; 2,277,013; 2,297,691; 2,357,809; 2,551,582; 2,825,814; 2,833,648; 3,220,324; 3,220,831; 3,220,833 and many others. Generally, these processes have in common the steps of employing a normally insulating photoconductive element which is prepared to respond to imagewise exposure with electromagnetic radiation by forming a latent electrostatic charge image. A variety of subsequent operations, now well known in the art, can then be employed to produce a permanent record of the image.

One type of photoconductive insulating structure or element particularly useful in electrophotography utilizes a composition containing a photoconductive insulating material dispersed in a resinous material. A unitary electrophotographic element is generally produced in a multilayer type of structure by coating a layer of the photoconductive composition onto a film support previously overcoated with a layer of conducting material or the photoconductive composition can be coated directly onto a conducting support of metal or other suitable conducting material. Such photoconductive compositions have shown improved speed and/or spectral response, as well as other desired electrophotographic characteristics when one or more photosensitizing materials or addenda are incorporated into the photoconductive composition. Typical addenda of this latter type are disclosed in U.S. Pat. Nos. 3,250,615; 3,141,770 and 2,987,395. Generally photosensitizing addenda to photoconductive compositions are incorporated to effect a change in the sensitivity or speed of a particular photoconductor system and/or a change in its spectral response characteristics. Such addenda can enhance the sensitivity of an element to radiation at a particular wavelength or to a broad range of wavelengths where desired. The mechanism of such sensitization is presently not fully understood. The phenomenon, however, is extremely useful. The importance of such effects is evidenced by the extensive search currently conducted by workers in the art for compositions and compounds which are capable of photosensitizing photoconductor compositions in the manner described.

Usually the desirability of a change in electrophotographic properties is dictated by the end use contemplated for the photoconductive element. For example, in document copying applications the spectral electrophotographic response of the photoconductor should be capable of reproducing the wide range of colors which are normally encountered in such use. If the response of the photoconductor falls short of these design criteria, it is highly desirable if the spectral response of the composition can be altered by the addition of photosensitizing addenda to the composition. Likewise various applications specifically require other characteristics such as the ability of the element to accept a high surface potential, and exhibit a low dark decay of electrical charge. It is also desirable for the photoconductive element to exhibit high shoulder speed and high toe speed as measured on an electrical H and D or characteristic curve, a low residual potential after exposure and resistance to fatigue. Electrical H and D curves as referred to herein are analogous to the curves first employed by Hurter and Driffield except that voltage or surface charge on the electrophotographic element is plotted instead of density. Sensitization of many photoconductive compositions and elements containing them by the addition of certain dyes selected from the large number of dyes presently known has hitherto been widely used to provide for the desired flexibility in the design of photoconductive elements in particular photocon-

ductive systems. Photoconductive compositions known to the art which are capable of exhibiting significant improvements in the aforementioned characteristics contain photosensitive addenda which are the subject of a copending application of William A. Light, titled NOVEL PHOTOCONDUCTIVE COMPOSITIONS AND ELEMENTS, Ser. No. 674,005, filed on Oct. 9, 1967, now abandoned. The addenda disclosed therein are responsible for the exhibition of desirable electrophotographic properties in photoconductive elements prepared therewith. Due to the need for supplying such elements, it has, therefore, become very important to establish the optimum conditions necessary for the most advantageous formation of the feature compositions so as to make maximum use of such material in the preparation of photoconductive elements.

It is, therefore, an object of this invention to provide the art of electrophotography with a novel method for the preparation of photoconductive compositions.

It is a further object of this invention to provide a new method for the formation of sensitizing addenda for use in electrophotographic compositions.

These and further objects and advantages of the present invention will become apparent from the following description and examples.

It has been discovered that many dyes and mixtures of dyes such as pyrylium dyes, including such pyrylium dyes as pyrylium, selenapyrylium and thiapyrylium dye salts can be combined with a wide variety of electrically insulating polymeric materials to form a separately identifiable multiphase heterogeneous composition of matter useful in electrophotography. The phases of the compositions are discernable under 2500X magnification. This novel composition is more particularly characterized in the previously described copending Light application. As disclosed by Light, the feature compositions can advantageously be formed in situ in a coated photoconductive layer by contacting the layer with the vapors of an organic composition which is capable of softening the layer (e.g., exposure to the vapors immediately adjacent to the surface of a bath of dichloromethane at 70° F.). It will be further described hereinafter according to this invention that excellent control of the production of the feature composition is now achieved by the use of novel shearing techniques applied to a solution containing a polymer and dye prior to coating. The photoconducting layers coated from dopes containing sheared constituents form the feature composition without the need for further treatment.

Typically, the preparation of the feature compositions according to this invention comprises preparing a coating dope by first mixing together the constituents of the composition until dissolved. At this point, a properly prepared dope should not contain any undissolved material and therefore appears homogeneous. Coatings subsequently prepared from such an untreated dope are also homogeneous and are rendered non-homogeneous only through the application of other preparatory means, such as vapor treatment, as disclosed by Light. In the practice of this invention, the coating of the homogeneous dope solution is preceded by the step of subjecting the solution to high speed shearing. Hereinafter, throughout the specification and claims such high speed shearing is intended to encompass stirring which is sufficiently vigorous to induce the formation of a multiphase composition of dye and polymer when the dope is coated. A multiphase heterogeneous composition containing aggregates visible under at least 2500X magnification is thereby formed in situ in the dried film without a vapor treatment of the cast layer as described by Light. Shearing the dope prior to coating thus eliminates the need for subsequent treatment of the dried film layer. It has further been discovered that varying the length of time of such shearing will vary the size of aggregates of the discontinuous phase formed subsequently in the cast layer and also increasing the shearing time produces a smaller sized aggregate which shows an increased electrophotosensitivity over photoconductive compositions having larger aggregates.

These results are quite unexpected when it is considered that the dope both before and after the shearing step remains as a homogeneous solution. No change appears to have taken place in the character of the solution which can be attributable to the shearing. It is, therefore, surprising that the sheared solution when coated will form an electrophotographic composition having properties not possessed by an unsheared solution. Likewise, while it would be expected that prolonged shearing would reduce the individual grain size of a dispersion of particles in a liquid medium, it is unexpected that an increase in the time of shearing can reproducibly reduce the size of the aggregate contained in the feature composition subsequently formed in a cast photoconductive layer. Equally surprising is the fact that small portions of a sheared solution, when added to a similarly constituted unsheared solution and then coated, will promote the formation of a multiphase heterogeneous composition having a predictable aggregate size depending upon the size of the aggregates from the original sheared solution. Varying the time of shearing of the original or seeding solution will likewise produce a variation in the aggregate size of the multiphase composition formed when a portion of the original sheared solution is added to a similarly constituted unsheared solution and coated. The phrase "similarly constituted" means only that the dye, for example, in the unsheared solution is of the same general class of pyrylium type dyes and not that the dye in the unsheared solution is necessarily identical to the dye of the sheared solution.

Observable heterogeneous structure in the present photoconductive layers is indicative of the presence of the feature compositions. The presence of such compositions in the layer permits the layer to produce the hereinafter enumerated improved properties when used as a photoconductor or as a photosensitizing addendum for other photoconductors. The feature compositions when formed in situ in a layer generally have an identifiable heterogeneous appearance when viewed under at least 2500X magnification, although such compositions may appear to be substantially optically clear to the naked eye in the absence of magnification. In other compositions prepared according to the invention, there is a macroscopic heterogeneity. Suitably, the dye-containing aggregate in the discontinuous phase is predominantly in the size range of about 0.01 to 25 microns. However, it should be noted that when the heterogeneous compositions of the invention are used to sensitize a particulate photoconductor, such as zinc oxide, another discontinuous phase will be present which may not fall within this size range.

In general, the present heterogeneous compositions are two phase organic solids containing dye and polymer. The polymer forms an amorphous matrix or continuous phase which contains a discrete discontinuous phase as distinguished from a solution. The discontinuous phase contains a significant portion of the dye present and generally a predominant portion of the dye present is in the discontinuous phase. The dye in the discontinuous phase can be considered as being in particulate form; however, that phase need not be comprised wholly of dye. It is believed that in some instances the discontinuous phase may be comprised of a cocrystalline complex of dye and polymer. However, it is also believed that all of the aggregates which can be formed by the process of this invention are not necessarily comprised of both dye and polymer. Preferably, substantially all of the dye present in the system is in the discontinuous phase. When the present compositions are used in conjunction with an organic photoconductor, the resultant photoconductive composition generally contains only two phases as the photoconductor usually forms a solid solution with the continuous polymer phase. On the other hand, when the multiphase compositions prepared as described herein are used in conjunction with a particulate photoconductor, three phases may be present. In such a case, there would be a continuous polymer phase, a discontinuous phase containing dye as discussed above and another discontinuous phase comprised of the particulate photoconductor. Of course, the present multiphase compositions may also contain additional discontinuous phases.

A photoconductive layer containing the feature composition prepared according to this invention has the same exceptional electrophotographic properties as the vapor-treated layers described in the previously identified copending application. For example, the layer which is formed after shearing differs in color from the color of a similar layer formed from an unsheared dope comprising the same constituents. That is, the layer cast from a dope comprising sheared materials absorbs radiation in a different wavelength region and spectrophotometrically records absorption maxima at different wavelengths than coatings prepared from unsheared solutions. The substantial shift in radiation absorption maximum when going from an unsheared to a sheared composition is generally of the magnitude of at least about 10 m $\mu$ . Similarly, a photoconductive layer prepared with the sheared dope has aggregates in the discontinuous phase normally visible under at least 2500X magnification and exhibits an increased electrophotographic speed. The dark conductivity of the compositions formed in accordance with the invention is often lowered, and a layer containing the compositions can often be repeatedly charged and exposed with substantially no apparent electrical fatigue. The observed tendency of elements containing materials prepared by this invention to recover very rapidly after charging and exposure is important in continuous or cyclic electrophotographic applications. When such compositions are present in an electrophotographic element, the element has improved regeneration properties or an improved ability to repeatedly accept a high surface potential after completion of a charge-expose-develop (or transfer) cycle. Likewise, such photoconductive layers do not have a memory and, therefore, do not retain spurious images between charging and exposing cycles.

The theoretical basis for the novel control that shearing accomplishes in the formation and physical appearance of feature compositions is at present not fully understood. The practical result achieved when shearing conditions are changed is useful and will be more fully described hereinafter. Based on the observed changes the shearing technique appears to be broadly applicable for accomplishing the formation of multiphase heterogeneous compositions from the many constituent materials capable of forming such compositions.

In the practice of this invention a wide variety of dyes and polymeric materials are capable of forming the feature compositions and can advantageously be utilized in the shearing process for the controlled formation of heterogeneous compositions. Typically, pyrylium dyes, including pyrylium, thiapyrylium and selenapyrylium dye salts are useful in the method of forming the compositions according to this invention. Such dyes include those which can be represented by the following formula:



wherein R<sup>a</sup>, R<sup>b</sup>, R<sup>c</sup>, R<sup>d</sup>, and R<sup>e</sup> can each represent (a) a hydrogen atom; (b) an alkyl group typically having from one to 15 carbon atoms, such as methyl, ethyl, propyl, isopropyl, butyl, tertiary butyl, amyl, isoamyl, hexyl, octyl, nonyl, dodecyl, etc., (c) alkoxy groups like methoxy, ethoxy, propoxy, butoxy, amyoxy, hexoxy, octoxy, and the like; and (d) aryl groups including substituted aryl groups such as phenyl, 4-diphenyl, alkylphenyls as 4-ethylphenyl, 4-propylphenyl, and the like, alkoxyphenyls as 4ethoxyphenyl, 4-methoxyphenyl, 4-amyloxyphenyl, 2-hexaoxyphenyl, 2-methoxyphenyl, 3,4-dimethoxyphenyl, and the like,  $\beta$ -hydroxy alkoxyphenyls as 2-hydroxyethoxyphenyl, 3-hydroxyethoxyphenyl, and the like, 4-hydroxyphenyl, halophenyls as 2,4-dichlorophenyl, 3,4-dibromophenyl, 4-chlorophenyl, 2,4-dichlorophenyl, and the like, azidophenyl, nitrophenyl, aminophenyls as 4-

diethylaminophenyl, 4-dimethylaminophenyl and the like, naphthyl; and vinyl substituted aryl groups such as styryl, methoxystyryl, diethoxystyryl, dimethylaminostyryl, 1-butyl-4-p-dimethylaminophenyl-1,3-butadienyl, 62 -ethyl-4-dimethylamino- styryl, and the like; and where is a sulfur, oxygen or selenium atom, and Z<sup>1</sup> is an anionic function, including such anions as perchlorate, fluoroborate, iodide, chloride, bromide, sulfate, periodate, p-toluenesulfonate, and the like. In addition, the pair R<sup>a</sup> and R<sup>b</sup> as well as the pair R<sup>d</sup> and R<sup>e</sup> can together be the necessary atoms to complete an aryl ring fused to the pyrylium nucleus. Typical pyrylium dyes for use in the present invention are listed in table 1.

TABLE 1

| Compound Number | Name of Compound                                                                                              | 15 | 6                                                                                               |
|-----------------|---------------------------------------------------------------------------------------------------------------|----|-------------------------------------------------------------------------------------------------|
| 1               | 4-[4-bis(2-chloroethyl)aminophenyl]-2,6-diphenylthiapyrylium perchlorate                                      | 37 | 6-( $\beta$ -methyl-4-dimethylaminostyryl)-2,4-diphenylpyrylium fluoroborate                    |
| 2               | 4-(4-dimethylaminophenyl)-2,6-diphenylthiapyrylium perchlorate                                                | 38 | 6-(1-ethyl-4-p-dimethylaminophenyl-1,3-butadienyl)-2,4-diphenylpyrylium fluoroborate            |
| 3               | 4-(4-dimethylaminophenyl)-2,6-diphenylthiapyrylium fluoroborate                                               | 39 | 6-[ $\beta$ , $\beta$ -bis(4-dimethylaminophenyl)vinylene]-2,4-diphenylpyrylium fluoroborate    |
| 4               | 4-(4-dimethylamino-2-methylphenyl)-2,6-diphenylthiapyrylium perchlorate                                       | 40 | 6-(1-methyl-4-p-dimethylaminophenyl-1,3-butadienyl)-2,4-diphenylthiapyrylium fluoroborate       |
| 5               | 4-[4-bis(2-chloroethyl)aminophenyl]-2-(4-methoxyphenyl)-6-phenylthiapyrylium perchlorate                      | 41 | 4-(4-dimethylaminophenyl)-2,6-diphenylpyrylium perchlorate                                      |
| 6               | 4-(4-dimethylaminophenyl)-2,6-diphenylthiapyrylium sulfate                                                    | 42 | 2,6-bis(4-ethylphenyl)-4-phenylpyrylium perchlorate                                             |
| 7               | 4-(4-dimethylaminophenyl)-2,6-diphenylthiapyrylium-p-toluenesulfonate                                         | 43 | 2,6-bis(4-ethylphenyl)-4-methoxyphenylthiapyrylium fluoroborate                                 |
| 8               | 4-(4-dimethylaminophenyl)-2,6-diphenylpyrylium-p-toluenesulfonate                                             | 44 | 2,4,6-triphenylthiapyrylium perchlorate                                                         |
| 9               | 2-(2,4-dimethoxyphenyl)-4-(4-dimethylaminophenyl)benzo[b]pyrylium perchlorate                                 | 45 | 4-(4-methoxyphenyl)-2,6-diphenylthiapyrylium perchlorate                                        |
| 10              | 2,6-bis(4'-ethylphenyl)-4-(4-dimethylaminophenyl)thiapyrylium perchlorate                                     | 46 | 6-(4-methoxyphenyl)-2,4-diphenylthiapyrylium perchlorate                                        |
| 11              | 4-(4-dimethylaminophenyl)-2-(4-methoxyphenyl)-6-phenylthiapyrylium perchlorate                                | 47 | 2,6-bis(4-ethylphenyl)-4-phenylthiapyrylium perchlorate                                         |
| 12              | 4-(4-dimethylaminophenyl)-2-(4-ethoxyphenyl)-6-phenylthiapyrylium perchlorate                                 | 48 | 4-(4-methoxyphenyl)-2,4-diphenylthiapyrylium perchlorate                                        |
| 13              | 4-(4-dimethylaminophenyl)-2-(4-methoxyphenyl)-6-(4-methylphenyl)pyrylium perchlorate                          | 49 | 4-(2,4-dichlorophenyl)-2,6-diphenylthiapyrylium perchlorate                                     |
| 14              | 4-(4-diphenylaminophenyl)-2,6-diphenylthiapyrylium perchlorate                                                | 50 | 2,4,6-tri(4-methoxyphenyl)thiapyrylium perchlorate                                              |
| 15              | 2,4,6-triphenylpyrylium perchlorate                                                                           | 51 | 2,6-bis(4-ethylphenyl)-4-phenylthiapyrylium perchlorate                                         |
| 16              | 4-(4-methoxyphenyl)-2,6-diphenylpyrylium perchlorate                                                          | 52 | 4-(4-ethoxyphenyl)-2,6-bis(4-ethylphenyl)thiapyrylium perchlorate                               |
| 17              | 4-(2,4-dichlorophenyl)-2,6-diphenylpyrylium perchlorate                                                       | 53 | 6-(4-dimethylaminostyryl)-2,4-diphenylthiapyrylium perchlorate                                  |
| 18              | 4-(3,4-dichlorophenyl)-2,6-diphenylpyrylium perchlorate                                                       | 54 | 2,4,6-triphenylthiapyrylium sulfate                                                             |
| 19              | 2,6-bis(4-methoxyphenyl)-4-phenylpyrylium perchlorate                                                         | 55 | 4-(4-methoxyphenyl)-2,6-diphenylthiapyrylium fluoroborate                                       |
| 20              | 6-(4-methoxyphenyl)-2,4-diphenylpyrylium perchlorate                                                          | 56 | 2,4,6-triphenylthiapyrylium chloride                                                            |
| 21              | 2-(3,4-dichlorophenyl)-4-(4-methoxyphenyl)-6-phenylpyrylium perchlorate                                       | 57 | 2-(4-ethoxyphenyl)-4,6-diphenylthiapyrylium fluoroborate                                        |
| 22              | 4-(4-ethoxyphenyl)-2,6-bis(4-ethylphenyl)pyrylium perchlorate                                                 | 58 | 4-(4-ethoxyphenyl)-2,6-bis(4-ethylphenyl)thiapyrylium perchlorate                               |
| 23              | 4-(4-ethoxyphenyl)-2,6-bis(4-methoxyphenyl)pyrylium perchlorate                                               | 59 | 2,6-bis(4-ethylphenyl)-4-(4-methoxyphenyl)thiapyrylium perchlorate                              |
| 24              | 2,4,6-triphenylpyrylium fluoroborate                                                                          | 60 | 4-anisyl-2,6-bis(4-n-amyloxyphenyl)thiapyrylium chloride                                        |
| 25              | 2,6-bis(4-ethylphenyl)-4-(4-methoxyphenyl)pyrylium perchlorate                                                | 61 | 2-[ $\beta$ , $\beta$ -bis(4-dimethylaminophenyl)vinylene]-4,6-diphenylthiapyrylium perchlorate |
| 26              | 2,6-bis(4-ethylphenyl)-4-methoxyphenylpyrylium fluoroborate                                                   | 62 | 6-( $\beta$ -ethyl-4-dimethylaminostyryl)-2,4-diphenylthiapyrylium perchlorate                  |
| 27              | 6-(3,4-dieethoxystyryl)-2,4-diphenylpyrylium perchlorate                                                      | 63 | 2-(3,4-dieethoxystyryl)-4,6-diphenylthiapyrylium perchlorate                                    |
| 28              | 6-(3,4-dieethoxy- $\beta$ -amylstyryl)-2,4-diphenylpyrylium fluoroborate                                      | 64 | 2,4,6-trianisylthiapyrylium perchlorate                                                         |
| 29              | 6-(4-dimethylamino- $\beta$ -ethylstyryl)-2,4-diphenylpyrylium fluoroborate                                   | 65 | 6-ethyl-2,4-diphenylpyrylium fluoroborate                                                       |
| 30              | 6-(1-n-amylo-4-p-dimethylaminophenyl-1,3-butadienyl)-2,4-diphenylpyrylium fluoroborate                        | 66 | 2,6-bis(4-ethylphenyl)thiapyrylium chloride                                                     |
| 31              | 6-(4-dimethylaminostyryl)-2,4-diphenylpyrylium fluoroborate                                                   | 67 | 6-( $\beta$ , $\beta$ -bis(4-dimethylaminophenyl)vinylene)-2,4-diphenylthiapyrylium perchlorate |
| 32              | 6-( $\alpha$ -ethyl-6 <sub>2</sub> , $\beta$ -dimethylaminophenyl vinylene)-2,4-diphenylpyrylium fluoroborate | 68 | 2,6-bis(4-ethylphenyl)-4-(4-ethoxyphenyl)thiapyrylium perchlorate                               |
| 33              | 6-(1-butyl-4-p-dimethylaminophenyl-1,3-butadienyl)-2,4-diphenylpyrylium fluoroborate                          | 69 | 6-(3,4-dieethoxy- $\beta$ -ethylstyryl)-2,4-diphenylpyrylium fluoroborate                       |
| 34              | 6-(4-dimethylaminostyryl)-2,4-diphenylpyrylium perchlorate                                                    | 70 | 6-(4-ethoxy- $\beta$ -ethylstyryl)-2,4-diphenylpyrylium fluoroborate                            |
| 35              | 6-[ $\beta$ , $\beta$ -bis(4-dimethylaminophenyl)vinylene]-2,4-diphenylpyrylium perchlorate                   | 71 | 2-(4-ethylphenyl)-4,6-diphenylthiapyrylium perchlorate                                          |
| 36              | 2,6-bis(4-dimethylaminostyryl)-4-phenylpyrylium perchlorate                                                   | 72 | 2,6-diphenyl-4-(4-methoxyphenyl)thiapyrylium perchlorate                                        |
|                 |                                                                                                               | 73 | 2,6-diphenyl-4-(4-methoxyphenyl)thiapyrylium fluoroborate                                       |
|                 |                                                                                                               | 74 | 2,6-bis(4-ethylphenyl)-4-(4-n-amyloxyphenyl)thiapyrylium perchlorate                            |
|                 |                                                                                                               | 75 | 2,6-bis(4-methoxyphenyl)-4-(4-n-amyloxyphenyl)thiapyrylium perchlorate                          |
|                 |                                                                                                               | 76 | 2,4,6-tri(4-methoxyphenyl)thiapyrylium fluoroborate                                             |
|                 |                                                                                                               | 77 | 2,4-diphenyl-6-(3,4-dieethoxystyryl)pyrylium perchlorate                                        |
|                 |                                                                                                               | 78 | 4-(4-dimethylaminophenyl)-2-phenylbenzo[b]selenapyrylium perchlorate                            |
|                 |                                                                                                               | 79 | 2-(2,4-dimethoxyphenyl)-4-(4-dimethylaminophenyl)benzo[b]selenapyrylium perchlorate             |
|                 |                                                                                                               | 80 | 4-(4-dimethylaminophenyl)-2,6-diphenylselenapyrylium perchlorate                                |
|                 |                                                                                                               | 81 | 4-(4-dimethylaminophenyl)-2-(4-ethoxyphenyl)-6-phenylselenapyrylium perchlorate                 |
|                 |                                                                                                               | 82 | 4-[ $\beta$ -bis(2-chloroethyl)aminophenyl]-2,6-diphenylselenapyrylium perchlorate              |
|                 |                                                                                                               | 83 | 4-(4-dimethylaminophenyl)-2,6-diphenylselenapyrylium perchlorate                                |
|                 |                                                                                                               | 84 | 4-(4-dimethylamino-2-methylphenyl)-2,6-diphenylselenapyrylium perchlorate                       |
|                 |                                                                                                               | 85 | 3-(4-dimethylaminophenyl)naphtho[2,1- $\beta$ ]selenapyrylium perchlorate                       |
|                 |                                                                                                               | 86 | 4-(4-dimethylaminostyryl)-2-(4-methoxyphenyl)benzo[b]selenapyrylium perchlorate                 |

87 2,6-di(4-diethylaminophenyl)-4-phenylselenapyrylium perchlorate

Preferred pyrylium dyes used in forming the feature aggregates according to the present invention are pyrylium dye salts having the formula:



wherein:

R<sub>1</sub> and R<sub>2</sub> can each be phenyl radicals, including substituted phenyl radicals having at least one substituent chosen from alkyl radicals of from one to six carbon atoms and alkoxy radicals having from one to six carbon atoms;

R<sub>3</sub> can be an alkylamino-substituted phenyl radical having from one to six carbon atoms in the alkyl moiety including di-alkylamino-substituted and halogenated alkylamino-substituted phenyl radicals;

X can be an oxygen or a sulfur atom; and

Z<sup>-</sup> is the same as above.

While the pyrylium dyes are preferred in preparing the present two phase heterogeneous systems, other photographic spectral sensitizing dyes that activate light exposed areas of photographic compositions can be utilized in the hydrophobic polymer of the present system.

Electrically insulating film-forming polymers suitable for the formation of electrophotographic compositions containing the aggregates prepared by this invention include polycarbonates and polythiocarbonates, polyvinyl ethers, polyesters, poly- $\alpha$ -olefins, phenolic resins, and the like. Mixtures of such polymers can also be utilized. Such polymers include those which function in the formation of the aggregates as well as functioning as binders for the sensitizer and photoconductor. Typical polymeric materials from these classes are set out in table 2.

TABLE 2

| Number | Polymeric Materials                                                            |
|--------|--------------------------------------------------------------------------------|
| 1      | polystyrene                                                                    |
| 2      | poly(vinyltoluene)                                                             |
| 3      | poly(vinylanisole)                                                             |
| 4      | polychlorostyrene                                                              |
| 5      | poly- $\alpha$ -methylstyrene                                                  |
| 6      | polyacenaphthalene                                                             |
| 7      | poly(vinyl isobutyl ether)                                                     |
| 8      | poly(vinyl cinnamate)                                                          |
| 9      | poly(vinyl benzoate)                                                           |
| 10     | poly(vinyl naphthoate)                                                         |
| 11     | poly(vinyl carbazole)                                                          |
| 12     | poly(vinylene carbonate)                                                       |
| 13     | poly(vinyl pyridine)                                                           |
| 14     | poly(vinyl acetal)                                                             |
| 15     | poly(vinyl butyral)                                                            |
| 16     | poly(ethyl methacrylate)                                                       |
| 17     | poly(butyl methacrylate)                                                       |
| 18     | poly(styrene-co-butadiene)                                                     |
| 19     | poly(styrene-co-methyl methacrylate)                                           |
| 20     | poly(styrene-co-ethyl acrylate)                                                |
| 21     | poly(styrene-co-acrylonitrile)                                                 |
| 22     | poly(vinyl chloride-co-vinyl acetate)                                          |
| 23     | poly(vinylidene chloride-co-vinyl acetate)                                     |
| 24     | poly(4,4'-isopropylidenediphenyl-co-4,4'-isopropylidenedicyclohexyl carbonate) |
| 25     | poly(4,4'-isopropylidenebis(2,6-dibromophenyl) carbonate)                      |
| 26     | poly(4,4'-isopropylidenebis(2,6-dichlorophenyl) carbonate)                     |
| 27     | poly(4,4'-isopropylidenebis(2,6-dimethylphenyl) carbonate)                     |
| 28     | poly(4,4'-isopropylidenediphenyl-co-1,4-cyclohexylidimethyl carbonate)         |
| 29     | poly(4,4'-isopropylidenediphenyl terephthalate)                                |

30 poly(3,3'-ethylenedioxyphenyl thiocarbonate)  
 31 poly(4,4'-isopropylidenediphenyl carbonate-co-terephthalate)  
 32 poly(4,4'-isopropylidenediphenyl carbonate)  
 33 poly(4,4'-isopropylidenediphenyl thiocarbonate)  
 34 poly(2,2-butanobis-4-phenyl carbonate)  
 35 poly(4,4'-isopropylidenediphenyl carbonate-block-ethylene oxide)  
 36 poly(4,4'-isopropylidenediphenyl carbonate-block-tetramethylene oxide)  
 37 poly[4,4'-isopropylidenebis(2-methylphenyl)carbonate]  
 38 poly(4,4'-isopropylidenediphenyl-co-1,4-phenylene carbonate)  
 39 poly(4,4'-isopropylidenediphenyl-co-1,3-phenylene carbonate)  
 40 poly(4,4'-isopropylidenediphenyl-co-4,4'-diphenyl carbonate)  
 41 poly(4,4'-isopropylidenediphenyl-co-4,4'-oxydiphenyl carbonate)  
 42 poly(4,4'-isopropylidenediphenyl-co-4,4'-carboxyldiphenyl carbonate)  
 43 poly(4,4'-isopropylidenediphenyl-co-4,4'-ethylenediphenyl carbonate)  
 44 poly(4,4'-methylenebis(2-methylphenyl)carbonate)  
 45 poly[1,1-(p-bromophenylethane)bis(4-phenyl)carbonate]  
 46 poly(4,4'-isopropylidenediphenyl-co-sulfonyl bis(4-phenyl)carbonate)  
 47 poly[1,1-cyclohexane bis(4-phenyl)carbonate]  
 48 poly(4,4'-isopropylidenediphenoxymethyldimethylsilane)  
 49 poly(4,4'-isopropylidenebis(2-chlorophenyl)carbonate)  
 50 poly[ $\alpha$ ,  $\alpha$ ',  $\alpha$ '-tetramethyl-p-xylylene bis(4-phenyl carbonate)]  
 51 poly(hexafluoroisopropylidene-4-phenyl carbonate)  
 52 poly(dichlorotetrafluoroisopropylidene-4-phenyl carbonate)  
 53 poly(4,4'-isopropylidenediphenyl-4,4'-isopropylidenedibenzoate)  
 54 poly(4,4'-isopropylidenedibenzyl-4,4'-isopropylidenedibenzoate)  
 55 poly(4,4'-isopropylidenedi-1-naphthyl carbonate)  
 56 poly(4,4'-isopropylidene bis(phenoxy-4-phenyl sulfone))  
 57 acetophenone-formaldehyde resin  
 58 poly(4,4'-isopropylidene bis(phenoxyethyl)-co-ethylene terephthalate)  
 59 phenol-formaldehyde resin  
 60 polyvinyl acetophenone  
 61 chlorinated polypropylene  
 62 chlorinated polyethylene  
 63 poly(2,6-dimethylphenylene oxide)  
 64 poly(neopentyl-2,6-naphthalenedicarboxylate)  
 65 poly(ethylene terephthalate-co-isophthalate)  
 66 poly(1,4-phenylene-co-1,3-phenylene succinate)  
 67 poly(4,4'-isopropylidenediphenyl phenylphosphonate)  
 68 poly(m-phenylcarboxylate)  
 69 poly(1,4-cyclohexanedimethyl terephthalate-co-isophthalate)  
 70 poly(tetra-methylene succinate)  
 71 poly(phenolphthalein carbonate)  
 72 poly(4-chloro-1,3-phenylene carbonate)  
 73 poly(2-methyl-1,3-phenylene carbonate)  
 74 poly(1,1-bi-2-naphthyl thiocarbonate)  
 75 poly(diphenylmethane bis-4-phenyl carbonate)  
 76 poly(2,2-(3-methylbutane)bis-4-phenyl carbonate)  
 77 poly(2,2-(3,3-dimethylbutane)bis-4-phenyl carbonate)  
 78 poly(1,1-(1-naphthyl)bis-4-phenyl carbonate)  
 79 poly(2,2-(4-methylpentane)bis-4-phenyl carbonate)  
 80 poly[4,4'-(2-norbornylidene)diphenyl carbonate]  
 81 poly[4,4'-(hexahydro-4,7-methanoindan-5-yliidene)diphenyl carbonate]

65 Especially useful polymers for forming the present heterogeneous compositions are compounds number 28, 30-47, 49, 51, 53, 54 and 76-81 as listed in table 2 above.

Included among the preferred polymers used for preparing the two phase heterogeneous compositions of the invention including copolymers, are those linear polymers having the following recurring unit:



wherein:

$R_4$  and  $R_5$ , when taken separately, can each be a hydrogen atom, an alkyl radical such as methyl, ethyl, propyl, isopropyl, butyl, tertiary butyl, pentyl, hexyl, heptyl, octyl, nonyl, decyl and the like including substituted alkyl radicals such as trifluoromethyl, etc., and an aryl radical such as phenyl and naphthyl including substituted aryl radicals having such substituents as a halogen, alkyl radicals of from one to five carbon atoms, etc., and  $R_4$  and  $R_5$ , when taken together, can represent the carbon atoms necessary to form a cyclic hydrocarbon radical including cycloalkanes such as hexyl and polycycloalkanes such as norbornyl, the total number of carbon atoms in  $R_4$  and  $R_5$  being up to 19;

$R_6$  and  $R_7$  can each be hydrogen, an alkyl radical of from one to five carbon atoms or a halogen such as chloro, bromo, iodo, etc., and

$R_8$  is a divalent radical selected from the following:



Among the hydrophobic carbonate polymers particularly useful in accordance with this invention are polymers comprised of the following recurring unit:



wherein:

each R is a phenylene radical including halo substituted phenylene radicals and alkyl substituted phenylene radicals; and  $R_4$  and  $R_5$  are described above. Such compositions are disclosed, for example, in U.S. Pat. Nos. 3,028,365 and 3,317,466. Preferably polycarbonates containing an alkylidene diarylene moiety in the recurring unit such as those prepared with Bisphenol A and including polymeric products of ester exchange between diphenylcarbonate and 2,2-bis(4-hydroxyphenyl)propane are used in the practice of this invention. Such compositions are disclosed in the following U.S. Pat. Nos. 2,999,750; 3,038,874; 3,038,879; 3,038,880; 3,106,545; 3,106,546; and published Australian Pat. Specification No. 19575/56. A wide range of film-forming polycarbonate resins are useful, particularly completely satisfactory results are obtained when using commercial polymeric materials which are characterized by an inherent viscosity of about 0.5 to 0.6. In addition, a high molecular weight material such as a high molecular weight Bisphenol A polycarbonate can be very useful. Preferably, such high molecular weight materials have an inherent viscosity of greater than about one as measured in 1,2-dichloroethane at a concentration of 0.25 g./100 ml. and a temperature of about 25°C. The use of high molecular weight polycarbonate, for example, facilitates the formation of aggregate compositions having a higher dye concentration which results in increased speeds.

Liquids useful as solvents for preparing coating solutions to be used in the practice of this invention can include, for example, a number of organic solvents such as aromatic hydrocarbons like benzene and toluene, ketones like acetone and ethyl-methyl ketone, halogenated hydrocarbons, like methylene chloride and ethylene chloride, furans like tetrahydrofuran, alkyl and aryl alcohols like methyl and ethyl, and benzyl alcohol, as well as mixtures of such solvents.

The heterogeneous compositions prepared as described herein are electrically insulating in the dark such that they will retain in the dark an electrostatic charge applied to the surface thereof. In addition, as mentioned above, the present compositions are also photoconductive. This term has reference to the ability of such compositions to lose a retained surface charge in proportion to the intensity of incident actinic radiation. In general, the term "photoconductive" as used to describe the present heterogeneous compositions means that the amount of incident radiation energy in meter-candle-seconds required to cause a 100 volt reduction in retained surface potential is not greater than about 200 meter-candle-seconds.

The heterogeneous compositions prepared by this invention are typically coated onto a conventional conducting support such as paper (at a relative humidity above 20 percent) including paper made more conductive by various coating and/or sizing techniques or carrying a conducting layer such as a conducting metal foil, a layer containing a semiconductor dispersed in a resin, a conducting layer containing the sodium salt of a carboxyester lactone of maleic anhydride and a vinyl acetate polymer such as disclosed in U.S. Pat. Nos. 3,007,901 and 3,262,806, a thin film of vacuum deposited nickel, aluminum, silver, chromium, etc., a conducting layer as described in U.S. Pat. No. 3,245,833, such as cuprous iodide, and like kinds of conducting materials. Such conducting materials can be coated in any well-known manner such as doctor-blade coating, swirling, dip-coating, spraying, and the like. Other supports, including such photographic film bases as poly(ethylene terephthalate), polystyrene, polycarbonate, cellulose acetate, etc., bearing the above conducting layers can also be used. The conducting layer can be overcoated with a thin layer of insulating material selected for its adhesive and electrical properties before application of a photoconducting layer. Where desired, however, the photoconducting layer can be coated directly on the conducting layer where conditions permit to produce the unusual benefits described herein.

When the present two phase compositions are used as photoconductor compositions, useful results are obtained by using the described dyes in amounts of about one to about 50 percent by weight of the coating composition. When the present multiphase compositions are used as sensitizers for photoconductive coatings, useful results are obtained by using the described dyes in amounts of about 0.001 to about 30 percent by weight of the photoconductive coating composition, although the amount used can be widely varied. The upper limit in the amount of photoconductive composition present in a sensitized layer is determined as a matter of individual choice and the total amount of any photoconductor used will vary widely depending on the material selected, the electrophotographic response desired, the proposed structure of the photoconductive element and the mechanical properties desired in the element. Lesser amounts of the present feature material can be utilized as sensitizing amounts to increase the speed sensitivity of other photoconductors than amounts that would be used if the feature material were the only photoconductor present.

Coating thicknesses of a photoconductive composition containing the feature compositions of the invention can vary widely. Normally, a wet coating in the range from about 0.0005 inch to about 0.05 inch on a suitable support material is useful in the practice of the invention. The preferred range of wet coating thickness was found to be in the range from about 0.002 inch to about 0.03 inch.

The compositions made by the present invention can readily be used for enhancing the sensitivity and extending the spectral range of sensitivity of a variety of organic photoconductors and inorganic photoconductors including both n- and p-type photoconductors. For example, these heterogeneous compositions can be used in connection with organic, including organometallic photoconducting materials which have little or substantially no persistence of photoconductivity. Representative organo-metallic compounds are the organic derivatives of Group IIa, IVa, and Va metals such as those

having at least one amino-aryl group attached to the metal atom. Exemplary organo-metallic compounds are the triphenyl-p-dialkylaminophenyl derivatives of silicon, germanium, tin and lead, the tri-p-dialkylaminophenyl derivatives of arsenic, antimony, phosphorous, bismuth boron, aluminum, gallium, thallium and indium. Useful photoconductors of this type are described in copending Goldman and Johnson U.S. Pat. application Ser. No. 650,664, filed July 3, 1967 and Johnson application Ser. No. 755,711, filed Aug. 27, 1968.

An especially useful class of organic photoconductors is referred to herein as "organic amine" photoconductors. Such organic photoconductors have as a common structural feature at least one amino group. Useful organic photoconductors which can be spectrally sensitized in accordance with this invention include, therefore, arylamine compounds comprising (1) diaryl-amines such as diphenylamine, dinaphthylamine, N,N'-diphenyl-benzidine, N-phenyl-1-naphthylamine, N-phenyl-2-naphthylamine, N,N'-diphenyl-p-phenylenediamine, 2-carboxy-5-chloro-4'-methoxy-diphenylamine, anilinophenol, N,N'-di-2-naphthyl-p-phenylene-diamine, those described in Fox U.S. Pat. No. 3,240,597, issued Mar. 15, 1966, and the like, and (2) triarylamines including (A) nonpolymeric triarylamines, such as triphenylamine, N,N,N'-N'-tetraphenyl-m-phenylenediamine, 4-acetyltriphenylamine, 4-hexanoyltriphenylamine, 4-lauroyltriphenylamine, 4-hexyltriphenyl-amine, 4-dodecyltriphenylamine, 4,4'-bis(diphenylamino)benzil, 4,4'-bis(diphenylamino)benzophenone and the like, and (b) polymeric triarylamines such as poly[N,4'-(N,N', N'-triphenylbenzidine)], polyadipyltriphenylamine, polysebacyltriphenylamine, polydecamethylenetriphenylamine, poly-N-(4-vinylphenyl)diphenylamine, poly-N-(vinylphenyl)- $\beta$ ,  $\beta'$ -dinaphthylamine and the like. Other useful amine-type photoconductors are disclosed in U.S. Pat. No. 3,180,730, issued Apr. 27, 1965.

Useful photoconductive substances capable of being sensitized in accordance with this invention are disclosed in Fox U.S. Pat. No. 3,265,496, issued Aug. 9, 1966, and include those represented by the following general formula:



wherein T represents a mononuclear or polynuclear divalent aromatic radical, either fused or linear (e.g., phenyl, naphthyl, biphenyl, binaphthyl, etc.), or a substituted divalent aromatic radical of these types wherein said substituent can comprise a member such as an acyl group having from one to about six carbon atoms (e.g., acetyl, propionyl, butyryl, etc.), an alkyl group having from one to about six carbon atoms (e.g., methyl, ethyl, propyl, butyl, etc.), an alkoxy group having from one to about six carbon atoms (e.g., methoxy, ethoxy, propoxy, pentoxy, etc.), or a nitro group; M represents a mononuclear or polynuclear monovalent aromatic radical, either fused or linear (e.g., phenyl, naphthyl, biphenyl, etc. or a substituted monovalent aromatic radical wherein said substituent can comprise a member, such as an acyl group having from one to about six carbon atoms e.g., acetyl, propionyl, butyryl, etc.), an alkyl group having from one to about six carbon atoms (e.g., methyl, ethyl, propyl, butyl, etc.), an alkoxy group having from one to about six carbon atoms e.g. methoxy, propoxy, pentoxy, etc.), or a nitro group; Q can represent a hydrogen atom, a halogen atom or an aromatic amino group, such as MNH-; b represents an integer from one to about 12; and, R represents a hydrogen atom, a mononuclear or polynuclear aromatic radical, either fused or linear (e.g., phenyl, naphthyl, biphenyl, etc.), a substituted aromatic radical wherein said substituent comprises an alkyl group, an alkoxy group, an acyl group, or a nitro group, or a poly(4'-vinylphenyl) group which is bonded to the nitrogen atom by a carbon atom of the phenyl group.

Polyarylalkane photoconductors are particularly useful in producing the present invention. Such photoconductors are described in U.S. Pat. No. 3,274,000, French Pat. No. 75

1,383,461 and in copending application of Seus and Goldman titled PHOTOCOndUCTIVE ELEMENTS CONTAINING ORGANIC PHOTOCOndUCTORS, Ser. No. 627,857, filed Apr. 3, 1967, now U.S. Pat. No. 3,542,544. These photoconductors include leuco bases of diaryl or triaryl methane dye salts, 1,1,1-triarylalkanes wherein the alkane moiety has at least two carbon atoms and tetraarylmethanes, there being substituted an amine group on at least one of the aryl groups attached to the alkane and methane moieties of the latter two classes of photoconductors which are nonleuco base materials.

Preferred polyarylalkane photoconductors can be represented by the formula:



wherein each of D, E and G is an aryl group and J is a hydrogen atom, an alkyl group, or an aryl group, at least one of D, E and G containing an amino substituent. The aryl groups attached to the central carbon atom are preferably phenyl groups, although naphthyl groups can also be used. Such aryl groups can contain such substituents as alkyl and alkoxy typically having one to eight carbon atoms, hydroxy, halogen, etc., in the ortho, meta or para positions, ortho-substituted phenyl being preferred. The aryl groups can also be joined together or cyclized to form a fluorene moiety, for example. The amino substituent can be represented by the formula



wherein each L can be an alkyl group typically having one to eight carbon atoms, a hydrogen atom, an aryl group, or together the necessary atoms to form a heterocyclic amino group typically having five to six atoms in the ring such as morpholino, pyridyl, pyrrol, etc. At least one of D, E, and G is preferably p-dialkylaminophenyl group. When J is an alkyl group, such an alkyl group more generally has one to seven carbon atoms.

Representative useful polyarylalkane photoconductors include the compounds listed in table 3.

TABLE 3

| Compound Number | Name of Compound                                                                      |
|-----------------|---------------------------------------------------------------------------------------|
| 1               | 4,4'-benzylidene-bis(N,N-diethyl-m-toluidine)                                         |
| 2               | 4',4''-diamino-4-dimethylamino-2',2''-dimethyltriphenylmethane                        |
| 3               | 4',4''-bis(diethylamino)-2,6-dichloro-2',2''-dimethyltriphenylmethane                 |
| 4               | 4',4''-bis(diethylamino)-2',2''-dimethyltriphenylmethane                              |
| 5               | 2',2''-dimethyl-4,4',4''-tris(dimethylamino)triphenylmethane                          |
| 6               | 4',4''-bis(diethylamino)-4-dimethylamino-2',2''-dimethyltriphenylmethane              |
| 7               | 4',4''-bis(diethylamino)-2-chloro-2',2''-dimethyl-4,4''-dimethylaminotriphenylmethane |
| 8               | 4',4''-bis(diethylamino)-4-dimethylamino-2,2',2''-trimethyltriphenylmethane           |
| 9               | 4',4''-bis(dimethylamino)-2-chloro-2',2''-dimethyltriphenylmethane                    |
| 10              | 4',4''-bis(dimethylamino)-2',2''-dimethyl-4-methoxytriphenylmethane                   |
| 11              | bis(4-diethylamino)tetraphenylmethane                                                 |
| 12              | bis(4-diethylamino)tetraphenylmethane                                                 |
| 13              | 4',4''-bis(benzylethylamino)-2',2''-dimethyltriphenylmethane                          |
| 14              | 4',4''-bis(diethylamino)-2',2''-dimethyltriphenylmethane                              |
| 15              | 4,4'-bis(dimethylamino)-1,1,1-triphenylethane                                         |
| 16              | 1-(4-N,N-dimethylaminophenyl)-1,1-diphenylethane                                      |
| 17              | 4-dimethylaminotetraphenylmethane                                                     |

Another class of photoconductors useful in this invention are the 4-diarylamino-substituted chalcones. Typical compounds of this type are low molecular weight nonpolymeric ketones having the general formula:



wherein  $R_1$  and  $R_2$  are each phenyl radicals including substituted phenyl radicals and particularly when  $R_2$  is a phenyl radical having the formula:



where  $R_3$  and  $R_4$  are each aryl radicals, aliphatic residues of one to 12 carbon atoms such as alkyl radicals preferably having one to 4 carbon atoms or hydrogen. Particularly advantageous results are obtained when  $R_1$  is a phenyl radical including substituted phenyl radicals and where  $R_2$  is diphenylaminophenyl, dimethylaminophenyl or phenyl.

Other photoconductors which can be used with the present aggregate compositions include rhodamine B, malachite green, crystal violet, phenoxyaniline, cadmium sulfide, cadmium selenide, parachloronil, benzil, trinitrofluorenone, tetrinitrofluorenone, zinc oxide, etc.

The following table 4 comprises a partial listing of U.S. Patents disclosing a wide variety of organic photoconductive compounds and compositions which can be improved with respect to speed, sensitivity, and/or regeneration when incorporated into the feature compositions and elements of this invention.

TABLE 4

| Inventor          | U.S. Pat. No. |
|-------------------|---------------|
| Hoegl et al.      | 3,037,861     |
| Sues et al.       | 3,041,165     |
| Schlesinger       | 3,066,023     |
| Bethe             | 3,072,479     |
| Klupfel et al.    | 3,047,095     |
| Neugebauer et al. | 3,112,197     |
| Cassiers et al.   | 3,133,022     |
| Schlesinger       | 3,144,633     |
| Noe et al.        | 3,122,435     |
| Sues et al        | 3,127,266     |
| Schlesinger       | 3,130,046     |
| Cassiers          | 3,131,060     |
| Schlesinger       | 3,139,338     |
| Schlesinger       | 3,139,339     |
| Cassiers          | 3,140,946     |
| Davis et al.      | 3,141,770     |
| Ghys              | 3,148,982     |
| Cassiers          | 3,155,503     |
| Cassiers          | 3,158,475     |
| Tomanek           | 3,161,505     |
| Schlesinger       | 3,163,530     |
| Schlesinger       | 3,163,531     |
| Schlesinger       | 3,163,532     |
| Hoegl             | 3,169,060     |
| Stumpf            | 3,174,854     |
| Klupfel et al.    | 3,180,729     |
| Klupfel et al.    | 3,180,730     |
| Neugebauer        | 3,189,447     |
| Neugebauer        | 3,206,306     |
| Fox               | 3,240,597     |
| Schlesinger       | 3,257,202     |
| Sues et al.       | 3,257,203     |
| Sues et al.       | 3,257,204     |
| Fox               | 3,265,496     |
| Kosche            | 3,265,497     |
| Noe et al.        | 3,274,000     |

The compositions of the present invention can be employed in photoconductive elements useful in any of the well-known electrophotographic processes which require photoconductive layers. One such process is the xerographic process. In a

- process of this type, an electrophotographic element held in the dark is given a blanket electrostatic charge by placing it under a corona discharge to give a uniform charge to the surface of the photoconductive layer. This charge is retained by the layer owing to the substantial dark insulating property, i.e., the low conductivity of the layer in the dark. The electrostatic charge formed on the surface of the photoconductive layer is then selectively dissipated from the surface of the layer by imagewise exposure to light by means of a conventional exposure operation such as, for example, by a contact-printing technique, or by lens projection of an image, and the like, to thereby form a latent electrostatic image in the photoconductive layer. Exposing the surface in this manner forms a pattern of electrostatic charge by virtue of the fact that light energy striking the photoconductor causes the electrostatic charge in the light struck areas to be conducted away from the surface in proportion to the intensity of the illumination in a particular area.

The charge pattern produced by exposure is then developed or transferred to another surface and developed there, i.e., either the charged or uncharged areas rendered visible, by treatment with a medium comprising electrostatically responsive particles having optical density. The developing electrostatically responsive particles can be in the form of a dust, i.e.,

powder, a pigment in a resinous carrier, i.e., toner. A preferred method of applying such toner to a latent electrostatic image for solid area development is by the use of a magnetic brush. Methods of forming and using a magnetic brush toner applicator are described in the following U.S. Pat. Nos.

2,786,439; 2,786,440; 2,786,441; 2,811,465; 2,874,063; 2,984,163; 3,040,704; 3,117,884; and Reissue 25,779. Liquid development of the latent electrostatic image may also be used. In liquid development the developing particles are carried to the image-bearing surface in an electrically insulating liquid carrier. Methods of development of this type are widely known and have been described in the patent literature, for example, U.S. Pat. No. 2,296,691 and in Australian Pat. No. 212,315. In dry developing processes the most widely used

method of obtaining a permanent record is achieved by selecting a developing particle which has as one of its components a low-melting resin. Heating the powder image then causes the resin to melt or fuse into or on the element. The powder is, therefore, caused to adhere permanently to the surface of the photoconductive layer. In other cases, a transfer of the charge

image formed on the photoconductive layer can be made to a second support such as paper which would then become the final print after development and fusing. Techniques of the type indicated are well known in the art and have been

described in a number of U.S. and foreign patents, such as U.S. Pat. No. 2,297,691 and 2,551,582 and in "RCA Review," Vol. 15 (1954) pages 469-484.

Processes such as described hereinbefore have found utility where the photoconductive layer is either inexpensive and expendable such as the various processes using photoconductive zinc oxide, or where the photoconductive media is rapidly reusable such as vitreous selenium. Many of the feature compositions of this invention now permit a large number of

known photoconductive compounds and compositions to be employed in xerographic processes where rapid repeated charging and exposing is desired.

The method of this invention is typically practiced as described in detail in the following examples.

## EXAMPLE 1

A photoconductive coating composition is prepared by dissolving 300 g. of a polycarbonate resin, a composition formed from the reaction between phosgene and a dihydroxydiarylal-kane or from the ester exchange between diphenylcarbonate

and 2,2-bis-4-hydroxyphenylpropane (Lexan 105 polycarbonate resin, General Electric Company), 200 g. of 4,4'-benzylidene bis (N,N-diethyl-m-toluidine) and 10 g. of 4-(4-dimethylaminophenyl)-2,6-diphenylthiapyrylium perchlorate in 1700 g. of methylene chloride and 1133.3 g. of 1,1,2-trichloroethane. This mixture is thoroughly dissolved after 2 hours of stirring. The resulting solution is then sheared by placing the solution in a high-speed shearing blender and shearing for a period of time. Samples of the solution are withdrawn from the blender at various times during the shearing and each sample is coated at a dry coverage of 0.7 g./ft.<sup>2</sup> from an extrusion hopper. The coating from the hopper is laid on a polyester film support which has previously been over-coated with two other layers. The layer next to the film support is a conducting layer comprising cuprous iodide in a resin binder. The layer overcoating the conducting layer is an insulating barrier layer of cellulose nitrate. After drying the separate coatings are visually examined. Each of the coatings shows the characteristic color and granular appearance of the formation of the feature composition. This examination also reveals that the samples which have undergone longer shearing times formed coatings having smaller aggregates than the aggregates formed in coatings prepared from dopes which have been sheared for shorter periods of time. In addition, increasing the length of time of shearing produces a change in the electrophotographic speeds of the various coatings. These speed changes are summarized in table 5. The actual positive

TABLE 5

| 5        | Sample<br>shearing<br>time,<br>minutes | Aggregate size<br>(microns) | Speed    |       |           |       |
|----------|----------------------------------------|-----------------------------|----------|-------|-----------|-------|
|          |                                        |                             | Shoulder |       | 50 v. toe |       |
|          |                                        |                             | Pos.     | Neg.  | Pos.      | Neg.  |
| (1)..... | 15                                     | 5.....                      | 5,700    | 6,500 | 80        | 1,800 |
| (2)..... | 30                                     | 4.....                      | 7,000    | 6,300 | 1,600     | 1,800 |
| (3)..... | 45                                     | 8.....                      | 8,000    | 6,300 | 2,000     | 2,000 |
| (4)..... | 60                                     | 1 to 2.....                 | 8,000    | 6,300 | 2,000     | 2,000 |
| (5)..... | 90                                     | .5 to 1.....                | 8,000    | 6,300 | 2,000     | 2,000 |
| (6)..... | 120                                    | About .1 to .2.....         | 8,000    | 6,300 | 2,000     | 2,000 |

## EXAMPLE 2

A solution prepared as described in example 1 is divided into three equal parts prior to shearing. For purposes of identification two of the parts (a) and (b) are not sheared prior to coating. The third part (c) is sheared for 4 hours in a high speed blender as in example 1 prior to coating. To insure the formation of multiphase heterogeneous composition in each case the coatings from (a) and (b) are vapor treated for 5 and 2 minutes respectively in the vapors of a bath of dichloroethane at 70° F. The results of aggregate size measurement after the various treatments, the electrophotographic shoulder and toe speed and the resolving power in lines per millimeter of the coatings when charged, exposed to a positive microimage and developed with a liquid developer in the manner described in U.S. Pat. No. 2,907,674 are recorded in table 6.

TABLE 6

| Solution<br>used | Shearing<br>time, hours | Aggregate<br>size<br>(microns) | Speed    |       |           |       |
|------------------|-------------------------|--------------------------------|----------|-------|-----------|-------|
|                  |                         |                                | Shoulder |       | 50 v. toe |       |
|                  |                         |                                | Pos.     | Neg.  | Pos.      | Neg.  |
| (a).....         | None                    | 5 to 10.....                   | 7,000    | 7,000 | 10        | 1,800 |
| (b).....         | None                    | 1 to 2.....                    | 8,000    | 6,300 | 1,800     | 1,700 |
| (c).....         | 4                       | About 0.1.....                 | 8,000    | 5,700 | 2,000     | 1,800 |

1/mm.

or negative electrical speeds of the coatings (as shown in table 5) are determined in the following manner. An element as described above is electrostatically charged under a corona source until the surface potential, as measured by an electrometer probe, reaches about 600 volts, positive or negative. The charged element is then exposed to a 3000° K. tungsten 40 light source through a stepped density gray scale. The exposure causes reduction of the surface potential of the element under each step of the neutral density scale from its initial potential,  $V_0$ , to some lower potential,  $V$ , whose exact value depends on the actual amount of exposure in meter-candle-45 seconds received by the area. The results of these measurements are then plotted on a graph of surface potential  $V$  vs. log exposure for each step. The actual positive speed of the element can then be expressed in terms of the reciprocal of the exposure required to reduce the surface potential to any arbitrarily selected value. Herein, unless otherwise stated, the actual electrical speed is the numerical expression of  $10^4$  divided by the exposure in meter-candle-seconds required to

50 The data recorded in table 6 clearly shows the effect of shearing on the formation of the heterogeneous composition in the coating and upon the electrophotographic properties of the coatings. Particularly advantageous is the observation that the formation of smaller aggregate sizes, which would be expected to promote higher resolution and optical clarity in the coating, also permits high electrophotographic speeds to be realized.

## EXAMPLE 3

A coating composition is prepared as in example 1 and divided into three parts prior to shearing. The separate compositions are sheared as in examples 1 and 2 for 30 min., 60 min., and 90 min. Each sheared composition is then added to separate unsheared solutions prepared in the same manner each comprising 10 times the volume of each sheared solution. The new solutions I, II and III contain, respectively, the 30 min. (I), 60 min. (II) and 90 min. (III) sheared constituents. Solutions I, II and III are coated as in example 1 and the results are recorded in table 7.

TABLE 7

| Solution   | Shear,<br>min. | Aggregate size<br>(microns) | Speed    |       |           |       |
|------------|----------------|-----------------------------|----------|-------|-----------|-------|
|            |                |                             | Shoulder |       | 50 v. toe |       |
|            |                |                             | Pos.     | Neg.  | Pos.      | Neg.  |
| (I).....   | 30             | 5.....                      | 7,000    | 6,300 | 20        | 2,000 |
| (II).....  | 60             | 1 to 2.....                 | 7,000    | 6,300 | 2,000     | 2,000 |
| (III)..... | 90             | About .1 to .2.....         | 7,000    | 6,300 | 2,000     | 2,000 |

1/mm.

reduce the 600 volt charged surface potential to a value of 500 volts (100 volt shoulder speed) or to 50 volts (50 volt toe speed). All of the sheared or heterogeneous coatings prepared as above can be toned to produce visible images after being charged and imagewise exposed, typical suitable toners being disclosed in U.S. Reissue Pat. No. 25,136.

70 The electrophotographic speed and resolution of the coatings reported in table 7 correspond closely to the results obtained where the entire coating dope was sheared prior to coating (see table 5). It is apparent from these results that the addition of small amounts of sheared material to a larger volume of material capable of forming a heterogeneous composition in

the coating, is sufficient to initiate such formation. It is also interesting to observe that the resultant aggregate size in the discontinuous phase of the dried coating is of the same order of magnitude as the aggregate size that could be expected from the shearing time of the added material. Close control of aggregate size within large volumes of coating dope can, therefore, be simply accomplished using sheared dope additions which have been classified by their ability to form certain sized aggregates.

#### EXAMPLE 4

The procedure of example 1 is generally repeated using as the sensitizer 0.4 g. of 4-(4-dimethylaminophenyl)-2,6-diphenylthiapyrylium perchlorate in place of the 4-[4-bis(2-chloroethyl)aminophenyl]-2,6-diphenylthiapyrylium perchlorate. The poly-carbonate resin, the photoconductor and the sensitizer are dissolved in a solvent mixture of 52.5 g. of dichloromethane and 52.5 g. of 1,2-dichloroethane by stirring the solids in the solvent for 2 hours at about 70° F. The resulting solution is then sheared for 20 minutes in a high speed shearing blender while maintaining the temperature of the solution at about 50° F. The sheared solution is then coated onto a conducting substrate. The substrate consists of an evaporated nickel film coated on Estar film base which is subbed with a terpolymer of 2 weight percent itaconic acid, 13 weight percent methyl acrylate and 85 weight percent vinylidene chloride. The net density of the evaporated nickel film is about 0.10 and the resistivity of the substrate is about 103 ohm./sq. This coating absorbs 94 percent of the incident radiation at the absorption peak of 675  $\mu$ . The electrophotographic element formed above is repeatedly charged to a positive or negative 600 v. potential and photodischarged to determine the resistance of the coating to electrical fatigue. After 1000 such cycles at a time interval of 3 seconds between photodischarging and recharging, the coating will still accept a high surface charge under the same charging conditions. This indicates that the coating has excellent regeneration properties. The positive and negative 100 v. toe speeds measured in a manner similar to that in example 1 are 3,200 and 3,500, respectively. The densities and resistivities of other metal conducting substrates such as titanium, nichrome, stainless steel, etc., as well as the regeneration properties, speeds and absorption of other organic photoconductive coatings which are coated directly on these metal substrates compare favorably with the above values.

#### EXAMPLE 5

Nine parts by weight of the polymer of example 1, six parts by weight of the photoconductor of example 1 and 0.3 parts by weight of the dye 4-(4-dimethylaminophenyl)-2,6-diphenylthiapyrylium fluoroborate are dissolved in 85 parts by weight of dichloromethane. Ten percent of the resultant solution is placed in a high shear blender and sheared for about one-half hour. The sheared solution is then added to the unsheared portion, thoroughly mixed and the combined solution is coated on a conducting support as in example 4. The dry thickness of the coating is about 10-12  $\mu$ . When viewed under magnification, the coating has a granular appearance. The resultant electrophotographic element is measured for speed as in example 1 with the exposure being changed slightly by the addition of a short wavelength pass interference filter having 30 percent transmittance at 600  $\mu$ . The negative 50 volt toe speed is 800 as compared to a speed of less than 50 for a similar element having a homogeneous coating of the same constituents which were not sheared.

#### EXAMPLE 6

A coating dope is prepared by dissolving 60 parts by weight of the binder of example 1, 40 parts by weight of the photoconductor of example 1 and four parts by weight of the dye 2-ethoxyphenyl-4-dimethylaminophenyl-6-phenylthiapyrylium perchlorate in methylene chloride with gentle stirring.

The dope is then coated as in example 1 to form a control element. Next, 100 parts by weight of the binder of example 1 and 0.015 parts by weight of the dye of example 1 are dissolved in methylene chloride and the solution is subjected to 5 high shear for a period of 30 minutes while maintaining the solution at 70° F. A 2 ml. portion of this sheared solution is added to a coating dope containing the constituents of the control followed by stirring. The combined solution is coated as above to form an electrophotographic element having an aggregate photoconductive layer thereon. The negative 100 v. toe speed of the element having the heterogeneous layer is 630 as compared to the negative 100 v. toe speed of 5.5 for the homogeneous control coating.

An improvement in electrophotographic properties similar to that shown in the preceding examples can be obtained when other dyes of the types described herein are incorporated into electrophotographic compositions prepared according to this invention. The control over the formation of the heterogeneous compositions as characterized herein is observed when these dyes are associated with polymeric materials according to the method of this invention. The heterogeneous compositions of this invention can readily be formed separately and then added to a suitable photoconductor. However, in order to reduce the necessary shearing time required to produce a given size aggregate, it is often advantageous to shear the dye and polymer in the presence of the photoconductor. In this manner, the shearing time can be reduced and the subsequent step of adding the heterogeneous composition to the photoconductor can be eliminated.

It will be apparent from the foregoing examples and description that the method of this invention permits the effective formation of electrophotographic compositions which can be utilized in photoconductive elements of many structural variations.

Likewise it should be apparent from the foregoing description and examples that no single form of shearing mechanism is essential for the effective preparation of heterogeneous compositions. Many commercially available high-speed shearing devices are well suited for use in practice of the present invention and exemplary devices are sold under such trade names as Gaulin Homogenizer, Cowles Dissolver, Premier Mill Dipersator, etc. The effectiveness of any device selected may be easily ascertained without undue experimentation by preparing sample coatings as described herein and inspecting the coatings for the formation of the feature compositions. Electrophotographic data will also help in determining the optimum combinations of conditions necessary to obtain the results desired.

The invention has been described in detail with particular reference to certain preferred embodiments thereof, but it will be understood that variations and modifications can be effected within the spirit and scope of the invention.

I claim:

1. A method for forming a heterogeneous photoconductive composition comprising the steps of dissolving in an organic solvent a pyrylium dye and polymeric material having an alkylidene diarylene moiety in the recurring unit, shearing said solution such that a coating prepared from said sheared solution is heterogeneous and absorbs radiation at a wavelength maximum at least 10  $\mu$  different from the wavelength of maximum absorption of an identical coating prepared from an unsheared solution containing the same constituents, forming a coating of said sheared solution, and drying said coating to form a heterogeneous composition comprising a continuous phase of said polymeric material and a discontinuous phase comprising a combination of said dye and polymeric material.

2. A method for producing a heterogeneous photoconductive insulating composition comprising the steps of preparing a solution of an electrically insulating polymeric material having an alkylidene diarylene moiety in the recurring unit and a pyrylium dye selected from the group consisting of pyrylium, thiapyrylium and selenapyrylium dye salts, subjecting said solution to high-speed shearing for an interval of time, coating

a thin layer of said solution and allowing said layer to dry to form a heterogeneous organic solid comprising a continuous phase of polymeric material having dispersed therein a discontinuous phase containing a combination of said polymeric material and dye, said shearing being performed for an interval of time at least sufficient to initiate the formation of a heterogeneous organic solid when coated and dried.

3. A method as described in claim 1 wherein electrically insulating polymeric material is a carbonate polymer and wherein said discontinuous phase is visible under at least 2500X magnification.

4. A method for preparing a heterogeneous photoconductive composition comprising the steps of dissolving in an organic solvent a pyrylium dye and an electrically insulating, film-forming polymeric material having an alkylidene diarylene moiety in the recurring unit, shearing the resultant solution at least until a test coating prepared from a portion of such solution forms a heterogeneous photoconductive layer having a maximum absorption at least 10 m $\mu$  different from the wavelength of maximum absorption of a test coating prepared from an unsheared portion of such solution, adding said sheared solution to a larger volume of a similarly constituted unsheared solution, coating the combined solutions and drying to form a heterogeneous composition comprising a continuous phase of polymeric material having dispersed therein a discontinuous phase comprising a combination of said dye and polymeric material.

5. A method for preparing an electrophotographic element comprising the steps of dissolving a pyrylium dye and a polycarbonate resin having an alkylidene diarylene moiety in the recurring unit in an organic solvent, shearing the resultant solution at least until a test coating prepared from a portion of said sheared solution forms a heterogeneous photoconductive layer having an absorption maximum at least 10 m $\mu$  different from the absorption maximum of a coating prepared from an unsheared portion of said solution, adding the sheared solution to a larger volume of a similarly constituted unsheared solution of a pyrylium dye and a polymeric material having an alkylidene diarylene moiety in the recurring unit, coating the combined solutions in a thin layer on a conductive support and drying said layer to form an electrophotographic element having a layer of a heterogeneous photoconductive composition comprising a continuous binder phase of polymeric material having dispersed therein a particulate discontinuous phase comprising a combination of said dye and polymeric material.

6. The method as described in claim 5 wherein the unsheared solution to which the sheared solution is added consists essentially of an organic solvent, a pyrylium dye, an electrically insulating, film-forming polymeric material having an alkylidene diarylene moiety in the recurring unit and an organic photoconductor.

7. The method of claim 1 wherein the electrically insulating polymeric material is a hydrophobic polymer having an alkylidene diarylene moiety in the recurring unit and wherein said discontinuous phase is visible under at least 2500X magnification.

8. The method of claim 1 wherein a photoconductive compound is added to said solution prior to shearing.

9. The method of claim 1 wherein the dye has the formula:

5



wherein:

R<sub>1</sub> and R<sub>2</sub> are aryl radicals selected from the group consisting of phenyl and substituted phenyl having at least one substituent selected from the group consisting of an alkyl radical of from one to six carbon atoms and an alkoxy radical of from one to six carbon atoms;

R<sub>3</sub> is an alkylamino-substituted phenyl radical having from one to six carbon atoms in the alkyl moiety;

X is selected from the group consisting of sulfur and oxygen; and

2<sup>1</sup> is an anion; and wherein the polymeric material contains the following recurring unit;



25 wherein:

R is a phenylene radical and each of R<sub>4</sub> and R<sub>5</sub>, when taken separately, is selected from the group consisting of a hydrogen atom, an alkyl radical of from one to 10 carbon atoms and a phenyl radical and R<sub>4</sub> and R<sub>5</sub>, when taken together, are the carbon atoms necessary to form a cyclic hydrocarbon radical, the total number of carbon atoms in R<sub>4</sub> and R<sub>5</sub> being up to 19.

10. The method of claim 1 wherein the dye is selected from 35 the group consisting of 4-(4-dimethylaminophenyl)-2,6-diphenylthiapyrylium perchlorate; 4-(4-dimethylaminophenyl)-2,6-diphenylthiapyrylium fluoroborate; 4-[4-bis(2-chloroethyl)aminophenyl]-2,6-diphenylthiapyrylium perchlorate; 4-(4-dimethylaminophenyl)-2,6-diphenylthiapyrylium 40 p-toluenesulfonate; 4-(4-dimethylaminophenyl)-2,6-diphenylpyrylium perchlorate; 4-(4-dimethylaminophenyl)-2,6-bis(4-ethylphenyl)thiapyrylium perchlorate; 4-(4-dimethylamino-2-methylphenyl)-2,6-diphenylpyrylium perchlorate 45 2-(4-methoxyphenyl)-4-[4-bis(2-chloroethyl)aminophenyl]-6-phenylthiapyrylium perchlorate; 2-(4-methoxyphenyl)-4-(dimethylaminophenyl)-6-phenylthiapyrylium perchlorate; 2-(4-ethoxyphenyl)-4-(dimethylaminophenyl)-6-phenylthiapyrylium perchlorate; 4-(4-dimethylaminophenyl)-2,6-diphenylthiapyrylium per 50 chlorate; and 4-(4-dimethylaminophenyl)-2,6-diphenylpyrylium p-toluenesulfonate.

11. The method of claim 3 wherein the dye of the sheared solution is selected from the group consisting of pyrylium and thiapyrylium dye salts and wherein the polymeric material of said sheared solution is a carbonate polymer.

12. The method of claim 3 wherein the unsheared solution to which the sheared solution is added comprises a solvent, a pyrylium dye, a hydrophobic polymer having an alkylidene diarylene moiety in the recurring unit and an organic photoconductor.

\* \* \* \* \*

UNITED STATES PATENT OFFICE  
CERTIFICATE OF CORRECTIONPatent No. 3,615,415 Dated October 26, 1971Inventor(s) Eugene P. Gramza

It is certified that error appears in the above-identified patent and that said Letters Patent are hereby corrected as shown below:

Column 18, line 62, delete "10 $\mu$ " and insert ---10 m $\mu$ ---.

Column 20, in the first formula, insert ---Z<sup>-</sup>---, as illustrated below:



Column 20, line 17, delete "2<sup>1</sup>" and insert ---Z<sup>-</sup>---; in the second formula, delete " $\approx$ " and insert therefor a single bond line line 55, after "salts" insert ---, wherein said unsheared solution contains a dye selected from the group consisting of pyrylium and thiapyrylium dye salts---.

Signed and sealed this 18th day of July 1972.

(SEAL)  
Attest:

EDWARD M.FLETCHER,JR.  
Attesting Officer

ROBERT GOTTSCHALK  
Commissioner of Patents